

D. J. FARMER.

MANUFACTURE OF NAILS.

No. 243,697.

Patented July 5, 1881.

*Fig 1.*



*Fig 3.*



*Fig 4.*



Inventor

David J. Farmer.

By *Knight Bros*  
attns.

Attest:

Geo. T. Smallwood Jr.  
Walter Allen

# UNITED STATES PATENT OFFICE.

DAVID J. FARMER, OF PENN YAN, NEW YORK, ASSIGNOR TO HIMSELF, JOHN P. FARMER, AND SAMUEL FARMER, OF SAME PLACE.

## MANUFACTURE OF NAILS.

SPECIFICATION forming part of Letters Patent No. 243,697, dated July 5, 1881.

Application filed August 29, 1879.

*To all whom it may concern:*

Be it known that I, DAVID J. FARMER, of Penn Yan, in the county of Yates, in the State of New York, have invented a new and useful 5 Improvement in the Manufacture of Cut Nails, of which the following is a specification.

My invention relates to the manufacture of cut nails by the use of what are generally known as "cut-nail machines," where nails are made 10 from the flat plate; and it consists in rolling sheets with a succession of transverse ridges forming inclined planes, cutting them up into nail-plates, converging from side to side in a direction longitudinal to the fiber of the metal, 15 cutting up the said plates (without the usual oscillation or inversion) into nail or tack blanks with the fiber lengthwise of the blank, and heading said blanks with customary or suitable cut-nail or tack machinery.

20 In order that my invention may be fully understood, I will proceed to describe it with reference to the accompanying drawings, in which—

Figure 1 represents a plan of my preferred 25 form of nail-plate as it comes from the rolls. Fig. 2 is a section of the same on the line 2 2, Fig. 1. Fig. 3 is a plan of a rolled plate of modified form, by which my invention may be carried into effect. Fig. 4 is a section on the 30 line 4 4, Fig. 3. Fig. 5 is a perspective view of a plate-section and of two nail-blanks severed therefrom, illustrating the mode of severing the blanks from the plate by straight parallel cuts.

35 In Figs. 1 and 2, A A represent ridges, and B B depressions, in the top of the rolled plate.

By my preferred mode of rolling the plate the ridges taper gradually in both directions, as shown in Figs. 1 and 2, from the lines a a 40 of greatest thickness to the lines b b of least thickness; but if preferred the taper may be made in one direction only, as illustrated in Figs. 3 and 4, in which case an abrupt or perpendicular shoulder is formed at each line a' a', 45 as represented in Fig. 4. The plates rolled in either mode are cut up into sections on the lines b b', and in the case of the oppositely-tapered plate shown in Figs. 1 and 2 on the lines a a' also. These plate-sections are intended to represent in width the length of

the nail, with additional length for the upsetting of the head, unless otherwise desired.

In my improvement, the taper desired for the nail being formed in the plate or iron before being fed into the machine, it is obvious that 55 it is only necessary, as before stated, to make a straight cut crosswise from the plate for each blank, or each nail made, so that in feeding the plate to the machine all that is required is to move the plate forward in a straight line to 60 the cutters of the machine, which may be done by weight, spring, or otherwise, as found desirable.

In the manufacture of the nails, the nails are cut and headed on the machine in the ordinary manner, cutting and heading the nail at one operation or revolution of the machine. I have not described the nail-machines, as they are well known and understood; and I do not confine my improvement to any precise form 70 of machine, as the forms and mechanisms of nail-machines are numerous and subject to change.

My improvement in cutting nails from the end of a taper plate and making a straight cut 75 crosswise from the plate saves one operation in the machine while making the nail, and will be readily understood to obviate the necessity heretofore of turning over the plate at each cut, or oscillating or changing the plate from 80 one pair of knives to another or its equivalent, to form the taper to the nail.

My improvement does not refer to forged 85 nails or spikes when the nail or spike is formed on the rod of iron point and head, which, when rolled or formed on the rod, is a continuous length of nails or spikes, to be separated one from the other after being made in a bar or continuous length. Neither does my improvement refer to a mode heretofore employed of 90 making forged nails by forming plates in a series of tapering sections or ridges, cutting up said plates transversely of the ridges, so as to produce strings of blanks point to head or point to point and head to head, and subsequently severing into separate blanks and finishing by hand-forging or otherwise, this mode having been described in a number of United States patents, some of them of old date. Neither does my improvement refer to the cut- 95 100

ting of tapering blanks from bars rolled with a transverse taper from edge to edge, as I am aware that this has before been proposed. It is manifest that with blanks cut from a bar 5 tapered transversely to the direction in which it is rolled the grain or fiber will be transverse to the blank, and hence cut nails can be successfully made by the process last referred to only by the use of homogeneous steel or iron 10 of the highest quality. My mode of rolling plates with transverse ridges and depressions, cutting these plates up into transversely-tapered bars, and cutting these up into blanks, produces nails with the grain or fiber lengthwise, as is necessary with the kind and quality 15 of iron commonly employed for nails.

I am aware that in the manufacture of horse-shoe-nails iron has been rolled into plates with ridges on one or both of their outer edges to 20 form the nail-heads, and with the fiber of the iron transverse to the plate or lengthwise with the nail; but such plates would not answer the purpose of my invention, and could not be used to form a tapered nail without inverting 25 or oscillating the plate at each cut.

I am also aware that plates have been rolled with an even taper transverse to the line of rolling, so that with fibrous iron nails cut from such plates would have the grain crosswise. This, therefore, I do not claim, as it necessitates the use of homogeneous iron and is not adapted for the manufacture of American cut 30 nails from common iron. 35

Having thus described my invention, the following is what I claim as new therein and desire to secure by Letters Patent:

As an improvement in the art of making cut nails and tacks, the process of rolling plates with transverse ridges and depressions, cutting these up into transversely-tapered 40 nail-plates with the fiber produced by previous rolling crosswise to said nail-plates, feeding such nail-plates to the nail-machine without the usual oscillation or alternate inversion, and heading in customary cut-nail or tack ma- 45 chinery, all substantially as set forth.

DAVID J. FARMER.

Witnesses:

S. FARMER,  
W. H. FARMER.